

CATION OF TEXTILES &amp; FIBERS,

10/30/34

## UNITED STATES PATENT OFFICE

1,978,800

METHOD FOR THE TREATMENT OF ANIMAL  
FURSKINS, ANIMAL HAIR FIBERS, AND  
THE LIKE

Gus Levy, New York, N. Y.

No Drawing. Application July 20, 1932,  
Serial No. 623,606

15 Claims. (Cl. 8—13)

This invention relates to a method of treating animal furskins and the like. More particularly, my invention relates to a method of preconditioning by which I obtain a furskin simulating a 5 genuine furskin of natural color and finish.

To those skilled in the furskin art, the fur which excels in quality is one which has a natural color, whose hair is of fine texture and lustre, and whose leather is strong, soft and at the same time 10 pliable. Such furskins are often rare and expensive. Heretofore, cheaper grades of furskins were subjected to certain processes in order that they might be used to imitate the rarer and more expensive furskins. These processes, however, 15 were expensive and difficult. The furskins were subjected to all sorts of chemical treatment which involved much time and expense, in order to obtain what was considered the desired result in the furskin.

20 Sometimes, due to such treatment, the leather was hard and brittle, or the hair was coarse, or was singed, thus producing a furskin of undesirable quality.

In many cases the mordants used in the chemical treatment thereof prior to bleaching were 25 inefficient and instead of improving the fur pelt and hair fibers, often impaired them or retarded the proper action of the dyeing solution, in which case the fur pelt was practically of no value.

30 Also, the bleaching treatment was a long and severe one. The furskins on being removed from the bleaching bath were in an exceedingly delicate condition, the pelt being very tender, and the hair fibers loose. This necessitated unusual 35 care in handling the furskins at this stage. Consequently after bleaching, the furskins had to be subjected to a redressing treatment in order to restore the lost properties originally inherent therein.

40 The process as generally used in the art also removed whatever mordanting chemicals had been absorbed by the hair fibers previous to bleaching. As a result, after bleaching and before dyeing, the furskins had to be remordanted 45 in order to obtain what was generally considered the proper result; namely, a furskin whose pelt is strong and at the same time soft and pliable and whose hair fibers are strong, of brilliant lustre and fine texture.

50 It is an object of the invention to provide an efficient method of treating animal furskins and the like, avoiding the aforementioned defects and disadvantages.

Another object of my invention is to provide a 55 method of economically producing a highly desir-

able furskin of unimpaired strength, fine texture and proper lustre, simulating a natural furskin of the color and finish characteristic of a normally good furskin and desirable to the trade.

A further object of my invention is to provide 60 a method of treating animal furskins and the like in which the hair fibers thereof contain, after a preliminary treatment, a mordant which will effectively accelerate a subsequent bleaching action, and which will effectively fix the dye if said 65 furskins are then subjected to a dyeing treatment. This mordant will also effectively fix the dye if the furskins are dyed without being subjected to a preliminary bleaching operation.

With the above objects and features in view my 70 invention in its essential form includes subjecting animal furskins and the like to the action of a solution which contains an alkali to cleanse and degrease the furskins and to open up the pores of the hair fibers, making them receptive to subsequent chemical treatment. At the same time the furskins are subjected to the action of a redressing solution to toughen the pelt and hair fibers in order to protect them from any injurious 75 effects of the subsequent treatments. The next 80 and important step is treating with a mordant solution containing complex ions of a metal and ammonia, to accelerate a subsequent bleaching action and to cause a fixation of the dye; if the furskins are to be dyed. The mordanted furskins 85 are then rinsed in water to eliminate any excess mordant solution, after which a bleaching and then a stripping action is performed. They may then be dyed if the color desired requires it. For 90 certain results the bleaching and stripping actions may be avoided and the furskins dyed directly after the mordanting.

While I have given above a somewhat general idea of the steps involved in my invention, I give 95 the following method described in detail as an illustrative example of carrying out my invention in the preferred form.

Furskins and the like, for instance rabbit skins are first washed in a solution containing: a 100 mild alkali such as sodium carbonate, in concentrations of from 0.05% to 5% and formaldehyde, in concentrations of from 0.05% to 2% for a period of about two (2) hours at ordinary temperatures. In this preliminary treatment there is both a "killing" and a "redressing" action. 105 The "killing" action of the alkali is to remove any adhering greases, fats or oils and to open up and clean out the pores of the hair fibers to render these hair fibers more susceptible to subsequent treatment. The "redressing" action of the 110

formaldehyde is to toughen the pelt and the hair fibers, thus offsetting any deleterious effects of the "killing" solution. It is to be noted that if the furskins remain too long in an ordinary "killing" 5 solution, particularly in the presence of high heat, the pelt and hair fibers become softened and soggy and unfit for subsequent treatments. The formaldehyde present in the solution toughens the pelt and strengthens the hair fibers and also 10 offsets any harmful effects of the "killing" solution. The formaldehyde also protects the pelt and the hair fibers against injurious effects of the bleaching agent in a step hereinafter described.

15 The furskins after treatment in the above step are now ready for a certain mordanting action, which is considered an important step in the present method. This action may also be considered for present purposes as a "fixing" action 20 in which the mordant or "fixer" reacts, apparently chemically, with the hair fibers of the furskins, thus preparing them for the bleaching and dyeing solutions. This treatment consists in introducing the mordanting chemicals into the hair 25 fibers. I have found that the type of mordants which produce the best results is of the chemical class of complex ions containing a metal and ammonia, represented by the formula



where  $M_{ex}$  represents a metal in any of its existing valences,  $(NH_3)_{2x}$  represents a number of 25 moles of ammonia equal to twice the valence of the metal and



represents the valence of the entire complex ion which is the same as the valence of the metal. The introduction of these complex metallic ammonia ions into the hair fibers is accomplished by subjecting the furskins to the action of a solution of a salt which consists of a positive radical of a metal in complex combination with ammonia, and a negative radical of any acid. Such a salt is ammonio-cupric sulphate  $Cu(NH_3)_4SO_4$ . While I prefer to use the above mentioned salt it is to be understood that any other salt of the same type may be used. That is, a salt consisting of a positive radical containing the metals copper, silver, cobalt, cadmium, nickel or zinc in complex combination with ammonia and a negative radical of any acid, such as sulphate, nitrate, chloride etc. The concentration of these mordanting salts may vary from 0.1% to 5%. The furskins are subjected to this mordanting action at ordinary temperatures for a period of from 1 to 8 hours, depending on the kind of furskins treated and the quality of the hair fibers, with their attendant adaptability to react with the mordanting solution. When the furskins have been subjected to this "mordanting" action for the desired period of time, they are rinsed with water to eliminate any excess of solution on the outside of the hair fibers.

For certain results the skins may now be dyed without any further preliminary treatment.

If lighter colors are desired the furskins are now bleached by treatment with a solution containing from 0.5% to 5% of either hydrogen peroxide, sodium peroxide, perborates, persulphates and the like, which will not, per se, color the hair fibers, and 5% sodium chloride, at ordinary tem-

peratures, for a period of from  $\frac{1}{2}$  to 2 hours, until the desired bleaching is obtained.

The furskins are now "stripped" with a solution containing about 1% of oxalic acid or any other acid and about 5% of sodium chloride at ordinary temperatures for a period of about one (1) hour, to remove a dark colored, curdy precipitate formed in the hair fibers during the bleaching action.

After this, the skins may be finished off in the ordinary manner, or they may be dyed and then finished off in the ordinary manner, depending on the color desired.

The use of sodium chloride in the bleaching and stripping actions while not absolutely necessary is preferable, as it prevents undue swelling of the pelt.

From the foregoing description of my invention it will be noted that I have described a highly efficient and economical method for the treatment of furskins and the like. In this method I can lengthen or shorten the time required for setting a furskin in the desired condition. I have also changed the physical and apparently the chemical constitution of the furskin pelt and hair 100 fibers by means of a mordanting solution containing complex metallic-ammonia ions, whereby the bleaching action has been greatly accelerated and the dye made fast to the hair fibers. However, it is to be understood that the dyeing step 105 is not an essential part of the process. If the color obtained by bleaching alone is satisfactory, the dyeing step may be avoided. It is also to be understood that in order to obtain certain color effects the bleaching and stripping actions 110 may be avoided and the furskins dyed directly after mordanting.

The furskins treated according to my invention, as herein described in its preferred form, have a fine texture, a smooth finish, are strong 115 and at the same time soft and pliable. The hair fibers after the chemical treatment hereinabove described are stronger and do not shed after use of the furskin. Also they retain the dye more tenaciously since there has been apparently a 120 chemical reaction between the fixing or mordanting agents and said hair fibers.

It is to be noted that according to my invention I am able to reduce appreciably the time consumed in treating a furskin, and at the same 125 time obtain a product which contains all the desirable features of a natural colored furskin. There is also a considerable economy of cost in the production of a furskin according to my invention, since the solution of one or more mordants may be re-used or if they are to be discarded, the metal salts and the ammonia may be recovered therefrom. A furskin which ordinarily 130 is of a dark or undesirable color or shade, or is of uneven color or shade can be treated according 135 to my invention without losing any of its desirable inherent characteristics, and at the same time the hair fibers and the pelt are improved in their quality, texture and appearance.

While I have described a preferred method of 140 treating furskins and the like, it is to be understood that various modifications or changes may be made as to steps, the quantities of reacting substances used, the temperatures, the time of treatment, or the changes in choice of mordants 145 of a complex metallic-ammonia ion character or their equivalents, without departing from the spirit and scope of my invention as defined in the following claims.

1. In the method of treating furskins and the 150

## TREATMENT &amp; CHEMICAL MODIFICATION OF TEXTILES &amp; FIBERS,

1,978,800

3

107

like, the steps including killing and redressing the furskins with a solution of sodium carbonate and formaldehyde, then treating same with a solution containing complex metallic ammonia ions, bleaching and then stripping the bleached furskins.

2. In the method of treating furskins and the like, the steps including killing and redressing the furskins with a solution of a basic substance and formaldehyde, then treating same with a solution containing complex metallic-ammonia ions, bleaching and then stripping the bleached furskins.

3. In the method of treating furskins and the like the steps including killing and redressing the furskins with a solution containing an alkali and formaldehyde, then treating same with a solution containing complex metallic-ammonia ions of the type.

20 
$$\left[ M_{2x} (NH_3)_{2x} \right]^y$$

where  $M_{2x}$  represents a metal in any of its existing valences,  $(NH_3)_{2x}$  represents a number of moles of ammonia equal to twice the valence of the metal, and  $y$  represents the valence of the entire complex metallic-ammonia ion which is the same as the valence of the metal; bleaching and then stripping the bleached furskins.

4. In the method of treating furskins and the like, the steps including killing and redressing the furskins with a solution containing an alkali and formaldehyde, treating same with a solution containing ammonio-cupric sulphate  $Cu(NH_3)_4SO_4$ , bleaching and then stripping the bleached furskins.

5. In the method of treating furskins and the like, the steps including killing and redressing the furskins with a solution containing an alkali and formaldehyde, treating same with a solution containing complex metallic-ammonia ions, bleaching with a solution containing hydrogen peroxide, then stripping the bleached furskins.

6. In the method of treating furskins and the like, the steps including killing and redressing the furskins with a solution containing an alkaline substance and formaldehyde, treating the same with a solution containing complex metallic-ammonia ions, bleaching the mordanted furskins with an oxidizing agent selected from the following group; persulphates, perborates, metallic peroxides; then stripping the bleached furskins.

7. In the method of treating furskins and the like, the steps including killing and redressing the furskins with a solution containing an alkali and formaldehyde, then treating same with a solution containing complex metallic-ammonia ions, bleaching the furskins, and then stripping them with a solution containing oxalic acid.

8. In the method of treating furskins and the like, the steps including killing and redressing the furskins with a solution containing a basic substance and formaldehyde, treating same with

a solution containing complex metallic-ammonia ions, bleaching and then stripping the bleached furskins with a solution containing an acid.

9. In the method of treating furskins and the like, the steps including killing the furskins with a solution containing an alkali, treating same with a solution containing complex metallic ammonia ions, bleaching and then stripping the bleached furskins.

10. In the method of treating furskins and the like, the steps including redressing the furskins with a solution containing formaldehyde, treating same with a solution containing complex metallic-ammonia ions, bleaching and finally 90 stripping the bleached furskins.

11. In the method of treating furskins and the like, the steps including subjecting the furskins to the action of a solution containing complex metallic-ammonia ions, and then bleaching the 95 same.

12. In the method of treating furskins and the like, the steps including subjecting the furskins to the action of a solution containing complex metallic-ammonia ions, bleaching, and then 100 stripping the bleached skins.

13. In the method of treating furskins and the like, the step which consists of mordanting the furskins or the like, preliminary to bleaching or dyeing, or both, by subjecting them to the 105 action of a solution containing complex metallic-ammonia ions, of the type represented by the formula

110 
$$\left[ M_{2x} (NH_3)_{2x} \right]^y$$

where  $M_{2x}$  represents a metal in any of its existing valences,  $(NH_3)_{2x}$  represents a number of moles of ammonia equal to twice the valence of the metal and

115

$$\left[ \quad \right]^y$$

represents the valence of the entire complex ion, which is the same as the valence of the metal.

120

14. In the method of treating furskins and the like, the step which consists of mordanting the furskins and the like, preliminary to bleaching or dyeing, or both, by subjecting them to the action of a solution containing ammonio-cupric 125 sulphate  $Cu(NH_3)_4SO_4$ .

15. In the method of treating furskins and the like, the step which consists of mordanting the furskins and the like, preliminary to bleaching or dyeing or both, by subjecting them to the 130 action of a solution containing a salt or salts whose positive radical consists of one of the following metals; copper, silver, cobalt, cadmium, nickel or zinc in complex combination with ammonia, and whose negative radical consists 135 of an acid radical.

GUS LEVY.

65

140

70

145

75

150